

## UNITED STATES PATENT OFFICE

FRANK W. HALL, OF PORT ARTHUR, TEXAS, ASSIGNOR, BY MESNE ASSIGNMENTS, TO  
THE TEXAS COMPANY, OF NEW YORK, N. Y., A CORPORATION OF DELAWARE

## ILLUMINATING OIL AND PROCESS OF MAKING SAME

No Drawing.

Application filed January 9, 1926. Serial No. 80,356.

This invention relates to improvements in illuminating oils and has particular reference to oils for use in railway signal lanterns and the like. The invention contemplates a process of preparing illuminating oils which includes compounding a kerosene or illuminating oil fraction of petroleum with a viscous highly purified hydrocarbon oil.

An important object of the invention is the preparation of an illuminating oil which will not flare up or die out when used in a signaling lantern under normal conditions of service, and which will burn for the required length of time in such a lantern without the formation of carbonaceous crusts upon the wick which would tend to lower or extinguish the flame.

In certain types of oil lamps, for example the hand lanterns used by railway men for signaling, it is necessary that a special oil having unusual properties shall be used. Such lanterns when used for signaling are often quickly raised and lowered or whirled about the head of the signalman so that there is a tendency for the oil to be either forced up the wick too rapidly or drawn down into the oil reservoir entirely, thus causing the flame to flare up and smoke the lantern globe or to die out to such an extent that the illumination is negligible.

The ordinary kerosene or burning oil fractions of petroleum are entirely unsuited for this purpose as they will not furnish a steady flame during the sudden movements of the signaling lantern, and in practice such oils are never used in this service. However, it has long been known that the compounding of a comparatively small proportion of a fatty oil, such for example as lard oil, with one of the heavier kerosene fractions of petroleum resulted in a signal oil having markedly improved burning qualities in that the tendency for the flame to fluctuate in height and intensity was considerably reduced. Although such compounded oils may be said to give fairly satisfactory service from the above-mentioned standpoint, they have the disadvantage of a tendency toward wick incrustation manifest by the formation of carbonaceous growths or deposits upon the

wick which may in a few hours completely extinguish the lantern in which the oil is being used. It is obvious that this is a serious matter in the case of railway signal lanterns which are required to give satisfactory 55 and uninterrupted service for as long as sixteen hours or more at a stretch.

Now I have discovered that by compounding a high grade kerosene oil or burning oil fraction of petroleum with a very highly 60 purified viscous hydrocarbon oil instead of the usual fatty oil, illuminating oils suitable for use in signal lanterns may be prepared which will give very superior service without wick incrustation and without substantial 65 fluctuation in the height of the flame during normal signaling operations.

In the preparation of such compounded signal oils it is essential that the viscous hydrocarbon oil shall be of the correct grade and 70 of the very highest degree of purity. The oil must be approximately water white in color and must not contain any asphaltic or tarry material or inorganic salts which might have a tendency to form a crust upon the lamp wick 75 during use. There are various methods of manufacturing white viscous hydrocarbon oils known to petroleum refiners such for example, as treating the oil with fuming sulfuric acid or with anhydrous aluminum chloride while under the influence of heat. However, for the production of the very pure viscous oils required for the purpose of manufacturing signal oils, I prefer to follow the procedure hereinafter described.

The petroleum, either of asphaltic or paraffin base, is subjected to distillation with steam or vacuum until a fraction having the desired properties as regards viscosity, flash point etc. is obtained. Such a portion of the oil may be an overhead distillate or a residuum as the qualities of the final product, due to the intensive purification to which the oil is subjected, are independent of this step in the refining process. The oil fraction, distilled to proper test, is then treated with sulfuric acid, the quantity of acid used varying with the particular type of oil which it is desired to refine. After the treatment with acid, the oil is subjected to further purification by up-

ward percolation through a column of fuller's earth or equivalent adsorbent material until rendered substantially colorless or water white. As an aid in the treating and filtering steps, the viscous oil may be diluted with a lighter petroleum fraction such as gasoline which is ultimately removed from the purified oil by distillation.

I wish to emphasize the fact that the passage of the oil through the column of fuller's earth is preferably upward or in a direction contrary to the forces of gravity for if the filtration is allowed to depend upon mere downward percolation, the oil will tend to "channel" and will not be wholly purified in its passage through the filter bed.

The limits of the physical characteristics of the viscous oil used in compounding signal oils may vary to a considerable degree; that is, the oil may be derived from naphthene or paraffin base crude petroleum and may be either a distillate or a residual product. The viscosity may range from say 400 seconds at 100° (Saybolt universal) to 200 seconds at 210° F. (Saybolt universal) but I have found that, in general a residual oil derived from a paraffin base crude petroleum refined by the above described preferred method and having approximately the following physical characteristics is most suitable for my purpose.

Viscosity ----- 100 to 150 seconds at 210° F.  
(Saybolt universal).

Color ----- Water white.  
Iodine value ----- Approximately zero.

Ash ----- None.

Thus, in the preparation of a signal oil according to my invention, a viscous oil of the type which I have just described is mixed with a high grade and highly purified heavy kerosene fraction of petroleum commonly known as 300 oil or mineral seal oil, in the proportion of from 5 to 40% or even more, although with an oil of this particular grade, I have found that approximately 25% by volume is the most satisfactory quantity to mix with the kerosene. The resulting oil is far better than that produced by using a fatty oil and as far as is known at present, is unequalled for service in signal lanterns.

Obviously many modifications and variations of the invention as hereinbefore set forth may be made without departing from the spirit and scope thereof, and therefore, only such limitations should be imposed as are indicated in the appended claims.

I claim:

1. An illuminating oil of the type adapted for feeding through a wick, comprising a mixture of a kerosene fraction of petroleum and a lesser proportion of a highly purified viscous hydrocarbon oil having a viscosity exceeding 100 seconds (Saybolt) at 210° F. adapted to modify the burning properties of the kerosene fraction, to furnish a uniform

burning flame without formation of substantial incrustation of the wick during use.

2. An illuminating oil of the type adapted for feeding through a wick, comprising a mixture of a kerosene fraction of petroleum and approximately 5 to 40 percent by volume of the mixture of a highly purified viscous hydrocarbon oil having a viscosity exceeding 100 seconds (Saybolt) at 210° F. adapted to modify the burning properties of the kerosene fraction, to furnish a uniform burning flame without formation of substantial incrustation of the wick during use.

3. An illuminating oil of the type adapted for feeding through a wick, comprising a mixture of a kerosene fraction of petroleum and a highly purified substantially water white hydrocarbon oil having a viscosity exceeding 100 seconds (Saybolt) at 210° F. and adapted to modify the burning properties of the kerosene fraction, to furnish a uniform burning flame without formation of substantial incrustation of the wick during use.

4. An illuminating oil of the type adapted for feeding through a wick, comprising a mixture of a kerosene fraction of petroleum and a highly purified substantially water white residual oil derived from a paraffin base crude petroleum, being adapted to modify the burning properties of the kerosene fraction, to furnish a uniform burning flame without formation of substantial incrustation of the wick during use.

In witness whereof I have hereunto set my hand this 30th day of December, 1925.

FRANK W. HALL

100

105

110

115

120

125

130